

## UNITED STATES PATENT OFFICE

2,654,709

COMPOUNDED HYDROCARBON OILS AND  
ADDITION AGENTS THEREFOR

Edward Mitchell, Pittsburgh, and Willard B. Morse, New Kensington, Pa., assignors to Gulf Research & Development Company, Pittsburgh, Pa., a corporation of Delaware

No Drawing. Application June 7, 1951,  
Serial No. 230,422

20 Claims. (Cl. 252—33.6)

1

This invention relates to addition agents for hydrocarbon lubricating oils in the nature of detergents and rust preventives. In particular the invention relates to new salt compositions. More particularly the invention is concerned with compounded hydrocarbon lubricating oils.

In the lubrication of internal combustion engines of all types, particularly when severe operating conditions are encountered, plain hydrocarbon lubricating oils frequently prove unsatisfactory in service. Furthermore, many lubricating oils which may be highly satisfactory for the lubrication of other mechanisms have been found wholly unsuitable for use as turbine oils.

Hydrocarbon lubricating oils are often objectionable because of deposition of sludge, carbonaceous materials, or varnish and because they fail to prevent the formation of rust. Consequently one or more addition agents are usually employed. For example, in order to counteract the tendency of lubricating oils to form deposits of gum and sludge, additives of a detergent nature are usually incorporated into such oils. To combat the formation of rust, rust-inhibiting agents are generally employed.

It is an object of this invention to provide an addition agent for hydrocarbon oils which functions both as a detergent and as a rust-preventive compound.

The lubricating compositions of the present invention comprise a hydrocarbon lubricating oil and a small amount of a polyvalent metal salt of the condensation product of an alkanethiol containing one to 17 carbon atoms with a monoamide of an unsubstituted or alkyl-substituted dicarboxylic acid as defined below. These metal salts are derivatives of 2,5-endoethylene- $\Delta^{3:4}$ -cyclohexene-1,6-dicarboxylic acid and the corresponding alkyl-substituted acids having not more than four alkyl groups each of not more than six carbon atoms. The N-substituents of the compounds are selected from hydrogen, alkyl and alkenyl radicals, and the total number of carbon atoms in the N-substituents is 8 to 22. At least one N-substituent must be an alkyl or alkenyl radical as defined.

The metal salts incorporated in hydrocarbon lubricating oils in accordance with the invention can be prepared in any suitable manner. We prefer, however, to prepare the alkanethiol-dicarboxylic acid monoamide condensation product and thereafter prepare the metal salt of this product. The reaction between the alkanethiol and the dicarboxylic acid monoamide is a conventional condensation reaction which results in the addition of an alkyl thio radical to one carbon

2

atom of an unsaturated linkage and hydrogen to the other carbon atom of this linkage. Thus, in cases where the N-substituents of the monoamide employed are either hydrogen and an alkyl radical or two alkyl radicals, the condensation product is a 2,5-endoethylene-alkyl thio-cyclohexane-1,6-dicarboxylic acid monoamide or the corresponding alkyl-substituted compound. The alkyl thio radical will be attached to the carbon atom in either the 3 or the 4 position of the cyclohexane ring.

In cases where the alkanethiol is condensed with a dicarboxylic acid monoamide having an alkenyl radical as an N-substituent, the condensation may take place either on the unsaturated linkage of the cyclohexene ring or on the unsaturated linkage of the alkenyl radical, and it is probable that condensation will take place on both unsaturated linkages.

It will be understood that the particular method of preparing the monoamide of the dicarboxylic acid employed for reaction with the alkanethiol forms no part of the present invention and that this compound can be prepared in any suitable manner. However, a preferred method of preparing the monoamide is disclosed in the copending application of Edward Mitchell, Serial No. 230,421, filed of even date herewith. The process as disclosed in the application comprises reacting a cyclohexadiene-1,3 compound with an alpha-beta ethylenic dicarboxylic acid containing not more than eight carbon atoms, such as maleic, citraconic, fumaric, glutaconic acids and their geometric isomers such as mesaconic acid and the like. Since the acids and the anhydrides are equivalents, the acids and the anhydrides are included when reference is made either to the acid or the anhydride unless otherwise indicated. The reaction between the cyclohexadiene-1,3 compound and the ethylenic dicarboxylic acid is essentially a Diels-Alder reaction. The resulting reaction product is then reacted with an amine under conventional amidating conditions to form the monoamide.

The diene compounds disclosed are cyclohexadiene-1,3,5-methyl cyclohexadiene-1,3, the dimethyl cyclohexadienes such as 4,6-dimethyl cyclohexadiene-1,3, and 2,4-dimethyl cyclohexadiene-1,3, the trimethyl cyclohexadienes such as 4,5,5-trimethyl cyclohexadiene-1,3, the methyl isopropyl cyclohexadienes such as alpha-terpinene, also 1,5-dimethyl-3-ethyl-cyclohexadiene-1,3, 1-methyl-3-ethyl-4-isopropyl cyclohexadiene-1,3, 1-methyl-5-isobutyl cyclohexadiene-1,3, and 1-methyl-5-n-hexyl cyclohexadiene-1,3. An alkyl-substituted 2,5-endoethylene- $\Delta^{3:4}$ -

cyclohexene-1,6-dicarboxylic acid prepared by the reaction between a cyclohexadiene-1,3 compound and an alpha-beta ethylenic dicarboxylic acid having an alkyl group attached to the carbon atom to which a carboxyl group is attached, will also contain an alkyl group attached to a carbon atom to which a carboxyl group is attached. It will be understood that all of the cyclohexene-1,6-dicarboxylic acids of this class which contain four alkyl groups must have one of these groups attached to a carbon atom to which a carboxyl group is attached. Moreover, such a carbon atom may contain an alkyl substituent in any case. For example, when cyclohexadiene-1,3 is condensed with citraconic acid, the resulting cyclohexene-1,6-dicarboxylic acid will contain one alkyl substituent and this a methyl group attached to a carbon atom to which a carboxyl group is also attached. Also, it will be noted that when an acid, such as glutaconic acid, in which the two carboxyl groups are not both attached to the carbon atoms forming the ethylenic double bond, is employed, the final cyclohexene dicarboxylic acid will be one in which a carboxyl group is linked to the cyclohexene ring through an alkylene radical. Such compounds are equivalent to those in which both carboxyl groups are attached directly to carbon atoms of the cyclohexene ring and are included when the 2,5-endoethylene- $\Delta^{3,4}$ -cyclohexene-1,6-dicarboxylic acids are referred to, unless otherwise indicated.

The amines which are employed in the formation of monoamides as disclosed in said copending application are primary alkyl or alkenyl amines having from 8 to 22 carbon atoms, and secondary alkyl and alkenyl amines having a total of from 8 to 22 carbon atoms. Examples of suitable amines are octyl amine, decyl amine, undecyl amine, dodecyl (lauryl) amine, tetradecyl amine, octadecyl amine, diamyl amine, dibutyl amine, N-butyl-decetyl amine, octenyl amine, decenyl amine, undecenyl amine, dodecenyl amine, tetradecenyl amine, hexadecenyl amine, and octadecenyl amine. Mixtures of amines such as are commercially available are desirable, for example mixtures of primary alkyl amines derived from fatty acids. These will be amines having approximately 8 to 22 carbon atoms.

In the preparation of the novel compounds in accordance with the present invention, the metal salt described in application U. S. Serial No. 230,421, can be condensed with an alkanethiol having 1 to 17 carbon atoms in the alkyl group. However, as stated above, it is preferred to start with the monoamide of the dicarboxylic acid mentioned supra. Without limiting ourselves to any theory we believe that since the alkanethiols are acidic in character the metal may be displaced in part if the metal salt is employed instead of the monoamide.

In preparing the metal salts of the instant invention by the methods mentioned above, equivalent amounts of the various reactants are preferably used. Thus about one mol of the diene, such as alpha-terpinene, can be reacted with about one mol of the acid, for example, maleic anhydride, at a temperature of from about 300° F. to about 340° F. The monoamide can then be prepared by adding about one mol of the amine at a temperature from about 180° F. to about 200° F. The alkanethiol derivative is preferably prepared by condensing said monoamide with about one mol of the alkanethiol. Where the

N-substituents are either hydrogen and an alkyl radical or two alkyl radicals there is no advantage in using more than one mol of the alkanethiol. However, when an alkenyl radical is an N-substituent, a larger amount of the alkanethiol can advantageously be used since, as pointed out previously, condensation may take place in the alkylene radical as well as in the cyclohexene ring. In condensing the alkanethiol with the monoamide so formed, it is generally desirable to employ a temperature of from about 100° F. to the boiling point of the particular alkanethiol employed. As an example, when 2-methylpropanethiol-1 is used, we prefer a temperature from about 100° F. to about 190° F., which is the boiling point of the 2-methyl-propanethiol-1. If the alkanethiol has a boiling point below about 100° F. as does methanethiol, it is necessary to carry out the reaction under pressure, for example, in an autoclave. In addition, it is obvious that if the boiling point of the alkanethiol is above the decomposition temperature of the monoamide, a temperature below said boiling point must be used. In this case, it is desirable to heat the reaction mixture at a temperature of from about 150° F. to about 160° F., usually for about one hour. The monoamide-alkanethiol condensation product so formed can then subsequently be neutralized with about one equivalent weight of a base such as barium hydroxide to form the metal salt.

The polyvalent metal salts can be prepared directly, that is, by neutralization or treatment with the metal oxide; or they can be prepared indirectly by double decomposition or metathesis. Desirable metals employed in the salt-forming reaction are barium, magnesium, calcium, nickel, zinc, lead, copper, strontium, aluminum, bismuth, iron, chromium and the like.

In some cases, selection of the particular alkanethiol may depend somewhat on steric hindrance. Thus, if a long chain amine was used it may be desirable to employ a short chain alkanethiol. While suitable alkanethiols will readily be known to those skilled in the art, the following are mentioned by way of example: methanethiol, ethanethiol, 1-propanethiol, 2-propanethiol, 1-butanethiol, 2-methyl-propanethiol-1, 1-pantanethiol, 3-pantanethiol, decanethiol, dodecanethiol, octanethiol and ceteanethiol.

When the unsaturated acid is contacted with the cyclohexadiene-1,3, some undesired polymer is normally formed. It is desirable to remove this polymer, which is conveniently accomplished by treatment of the final salts. The treatment preferably involves extraction with a solvent. The salts can be readily dissolved in common solvents such as benzene, Stoddard solvent, chloroform and light hydrocarbon oils. The solution is then filtered and, in the case of a volatile solvent, heated to evaporate said solvent. Inasmuch as oil concentrates of the salts of the present invention are desirable for use, it is preferred to extract the salt using a light hydrocarbon lubricating oil.

The following examples illustrate the various methods of preparing our improvement agents and improved compositions containing the same.

#### Example I

In this example 23.3 parts by weight of dipentene were heated to a temperature of from 300° F. to 340° F. for about 30 minutes to rearrange the double bonds in the dipentene molecule to form a conjugated system, the product

## 5

being alpha-terpinene, 1-methyl-4-isopropyl-cyclohexadiene-1,3. To this product 16.3 parts by weight of maleic anhydride were added. The reaction temperature was maintained at 300° F. to 320° F. for one hour. The temperature of the reaction mixture was then lowered to about 200° F. and 41.3 parts by weight of hexadecyl amine were added portion-wise. After completing the addition of the hexadecyl amine the reactants were maintained at a temperature of 180° F. to 220° F. for 30 minutes. The reactants were cooled to a temperature of from 150° F. to 160° F. and 15.4 parts by weight of tertiary butyl mercaptan were added, and the reaction temperature was maintained at 150° F. to 160° F. for one hour. At the end of the hour 3.5 parts by weight of magnesium oxide were added and the reactants were heated at about 180° F. for about one hour. The product was then extracted with a volatile solvent, filtered, and the solvent removed by distillation. The magnesium salt thus prepared had the following properties:

|                    |             |
|--------------------|-------------|
| Appearance         | Amber solid |
| Neutralization No. | 0.86        |
| Percent ash as MgO | 4.05        |
| Percent sulfur     | 1.70        |

## Example II

In this example 22.8 parts by weight of alpha-terpinene were heated to a temperature from 300° F. to 320° F. Then 16.7 parts by weight of maleic anhydride were slowly added and the heating continued at a temperature of 300° F. to 320° F. for one hour. The reactants were cooled to a temperature of from 200° F. to 210° F. and 41 parts by weight of a mixture of amines were added, the temperature being maintained at 200° F. to 210° F. for 30 minutes. The composition of the mixture of amines was 90% hexadecyl amine, 6% octadecyl amine, and 4% octadecenyl amine. To the monoamide so formed 15.3 parts by weight of n-butyl mercaptan were added and the mixture was heated to a temperature of from 150° F. to 160° F. for 60 minutes. Then, 4.2 parts by weight of magnesium oxide were added and the reaction mixture was agitated at a temperature of from 200° F. to 212° F. for at least 60 minutes. The magnesium salt so formed was extracted with a volatile solvent, filtered and the solvent removed by distillation.

## Example III

In this example 23.5 parts by weight of alpha-terpinene were heated to a temperature of 300° F. Then, 17.0 parts by weight of maleic anhydride were slowly added and the heating continued at a temperature of 300° F. to 320° F. for one hour. The reactants were cooled to a temperature of from 200° F. to 250° F. and 43.3 parts by weight of a mixture of amines were added, the temperature being maintained at 200° F. to 250° F. for 15 minutes. The composition of the mixture of amines was 90 per cent hexadecyl amine, 6 per cent octadecyl amine and 4 per cent octadecenyl amine. To the monoamide so formed 12.7 parts by weight of n-propanethiol were added and the mixture was heated to a temperature of from 150° F. to 160° F. for 60 minutes. Then, 3.5 parts by weight of magnesium oxide were added and the reaction mixture was agitated at a temperature of from 180° F. to 190° F. for at least 60 minutes. The magnesium salt so formed was extracted with a light hydrocarbon lubricating oil.

## 6

## Example IV

In this example, 20.7 parts by weight of alpha-terpinene were heated to a temperature from 300° F. to 320° F. Then 14.9 parts by weight of maleic anhydride were slowly added and the heating continued at a temperature of 300° F. to 320° F. for one hour. The reactants were cooled to a temperature of from 190° F. to 200° F. and 36.0 parts by weight of a mixture of amines were added, the temperature being maintained at 190° F. to 200° F. for 30 minutes. The composition of the mixture of amines was 25 per cent hexadecyl amine, 70 per cent octadecyl amine and 5 per cent octadecenyl amine. To the monoamide so formed, 13.9 parts by weight of tertiary butyl mercaptan were added and the mixture was heated to a temperature of from 150° F. to 155° F. for 60 minutes. Then, 4.3 parts by weight of barium oxide were added and the reaction mixture was agitated at a temperature of from 180° F. to 200° F. for at least 60 minutes. The barium salt so formed was extracted with a volatile solvent, filtered and the solvent removed by distillation.

## Example V

In this example, 22.7 parts by weight of alpha-terpinene were heated to a temperature from 310° F. to 320° F. Then, 16.6 parts by weight of maleic anhydride were slowly added and the heating continued at a temperature of 310° F. to 320° F. for one hour. The reactants were cooled to 200° F. and 41.4 parts by weight of a mixture of amines were added, the temperature being maintained at 200° F. for 30 minutes. The mixture of amines was composed of 90 per cent hexadecyl amine, 6 per cent octadecyl amine and 4 per cent octadecenyl amine. To the monoamide so formed, 15.2 parts by weight of tertiary butyl mercaptan were added and the mixture was heated to a temperature of 150° F. for 60 minutes. Then, 4.1 parts by weight of magnesium oxide were added and the reaction mixture was agitated at a temperature of from 210° F. to 215° F. for at least 60 minutes. The magnesium salt so formed was extracted with a volatile solvent, filtered and the solvent removed by distillation.

## Example VI

In this example, 47 parts by weight of alpha-terpinene were heated to a temperature from 300° F. to 320° F. Then, 34 parts by weight of maleic anhydride were slowly added and the heating continued at a temperature of 300° F. to 320° F. for one hour. The reactants were cooled to a temperature of from 200° F. to 210° F. and 100 parts by weight of a mixture of amines were added, the temperature being maintained at 200° F. to 210° F. for 30 minutes. The composition of the mixture of amines was 90 per cent hexadecyl amine, 6 per cent octadecyl amine and 4 per cent octadecenyl amine. To the monoamide so formed, 84 parts by weight of cetyl mercaptan were added and the mixture was heated to a temperature of from 150° F. to 160° F. for 60 minutes. Then, 7 parts by weight of magnesium oxide were added and the reaction mixture was agitated at a temperature of from 200° F. to 212° F. for at least 60 minutes. The magnesium salt so formed was extracted with a volatile solvent, filtered and the solvent removed by distillation.

The salts prepared in accordance with this invention are excellent addition agents for hy-

drocarbon lubricating oils. Concentrates can be readily prepared as described above and the salts can be added to lubricating oils in the form of such concentrates. Also, the salts can be added directly to the lubricating oil in the desired proportions. All types of hydrocarbon oils, including mineral oils, such as paraffinic, naphthenic, and mixed-base mineral oils, can be employed.

As stated, our new addition agents are remarkably effective in inhibiting rust and in improving detergent properties of hydrocarbon lubricating oil compositions. For this purpose small amounts of the addition agents are generally sufficient. For example, the addition agents of the instant invention may be added to hydrocarbon lubricating oils in minor amounts, say from 0.1 to 0.1 per cent by weight of the hydrocarbon oil, sufficient to inhibit rust formation. Larger amounts of our addition agent, from 0.1 to about

total of 216 operating hours has accrued. The piston varnish formation is compared with a set of prepared standards and given an Arbitrary Varnish Rating Value. The piston color is rated on this arbitrary scale which ranges from 10 (no varnish formed) to 0 (very heavy varnish formation) representing increasing discoloration of the piston skirt. The data obtained in these tests on the following compositions is summarized below. The percentages are by weight of the compositions.

|                                                                   | Composition I | Composition II | Composition III | Composition IV |
|-------------------------------------------------------------------|---------------|----------------|-----------------|----------------|
| Base Lubricating Oil, described above, percent.....               | 100.0         | 91.0           | 92.86           | 92.86          |
| Magnesium Salt prepared in accordance with Example II, percent... | 0.0           | 9.0            | 7.14            | 7.14           |

TABLE I

| Length of Test, Hours | Composition  |                     |              |                     |              |                     |              |                     |
|-----------------------|--------------|---------------------|--------------|---------------------|--------------|---------------------|--------------|---------------------|
|                       | I            |                     | II           |                     | III          |                     | IV           |                     |
|                       | Piston Color | No. of Struck Rings | Piston Color | No. of Struck Rings | Piston Color | No. of Struck Rings | Piston Color | No. of Struck Rings |
| 24.....               | 2+           | 0                   | 10           | 0                   | 10           | 0                   | 10           | 0                   |
| 48.....               | 0            | 1                   | 9            | 0                   | 9+           | 0                   | 10           | 0                   |
| 72.....               |              |                     | 5            | 0                   | 0            | 0                   | 9+           | 0                   |
| 96.....               |              |                     | 5            | 0                   | 0            | 0                   | 9+           | 0                   |
| 120.....              |              |                     | 5            | 0                   | 0            | 0                   | 9+           | 0                   |
| 144.....              |              |                     | 5            | 0                   | 0            | 0                   | 9+           | 0                   |
| 168.....              |              |                     | 5            | 0                   | 0            | 0                   | 8+           | 0                   |
| 192.....              |              |                     | 5            | 0                   | 0            | 0                   | 8+           | 0                   |
| 216.....              |              |                     | 5            | 0                   | 0            | 0                   | 8+           | 0                   |

<sup>1</sup> Mechanical failure.

20 per cent by weight of the hydrocarbon oil, confer excellent detergent properties on the oil solution. Table I following illustrates the remarkable detergent effects of the new addition agents. The oil employed as the base oil in these compositions was a solvent-refined Mid-Continent oil of lubricating grade having the following characteristics:

|                               |      |
|-------------------------------|------|
| Gravity, ° API.....           | 28.4 |
| Viscosity, SUS @ 100° F.....  | 464  |
| Viscosity, SUS @ 210° F.....  | 61.7 |
| Viscosity Index.....          | 98   |
| Flash point, ° F.....         | 480  |
| Pour point, ° F.....          | -5   |
| Sulfur, per cent.....         | 0.17 |
| Carbon residue, per cent..... | 0.06 |
| Neutralization No.....        | 0.03 |

These compositions were tested in a standard Lauson engine for their ability to prevent ring-sticking. This test consists in placing 2.1 pounds of the composition in the crankcase of the Lauson engine so modified and so operated as to make the conditions comparable to those prevailing in high-speed automotive-type diesel engines. The engine is operated under a 3 H. P. load at 1850 R. P. M. maintaining a cooling jacket temperature of 300° F., an oil temperature of 225° F. and an air-to-fuel ratio of 13:1. At the end of 24 hours operation under these conditions the engine is stopped, disassembled, and the piston is examined as to stuck rings and discoloration. If there are no stuck rings, the engine is reassembled, the oil charge is brought up to 2.1 pounds, and operation is continued for another 24-hour period. This procedure is repeated until one of the rings sticks or until a

total of 216 operating hours has accrued. Although the test on Composition III was stopped because of mechanical failure, it will be seen from these data that the addition to a typical crankcase lubricant of minor amounts of a magnesium salt prepared in accordance with this invention, effects a fourfold increase in the time required for ring-sticking to occur in a diesel engine. The tests show marked improvement in a ring-sticking and in piston color over the base oil.

In order to demonstrate the anti-rust properties of the compositions prepared in accordance with this invention, an oil containing a small amount of the magnesium salt was subjected to the test specified in the "ASTM Standards on Petroleum Products and Lubricants," September 1945, and designated as ASTM D-665-44T. In brief, the test consists in placing a 300 ml. sample of the oil or oil composition to be tested in a 400 ml. beaker which is immersed in a constant temperature bath maintained at 140° F. The beaker is fitted with a cover provided with openings for a stainless steel motor-driven stirrer and for insertion of a standard steel test bar, 1/2 inch in diameter and 5 1/2 inches long, which has been very carefully cleaned and polished just prior to the test. The stirrer is started, and when the oil sample in the beaker reaches a steady temperature of 140° F. the test bar is inserted in the proper opening and hangs suspended from the beaker cover. After 30 minutes, 30 ml. of distilled water are added to the beaker, and stirring is continued for 48 hours, after which time the test bar is removed and examined for rust spots. In carrying out this test 0.05 per cent by weight of the oil of the magnesium salt

prepared in accordance with Example I was used. The oil employed in the test was an aluminum chloride-treated paraffinic oil having a viscosity of 150 S. U. S. at 100° F. A test was carried out on the base oil, and on the base oil having said magnesium salt incorporated therein. No rust formed on the test bar in our inhibited oil even after 48 hours. The test bar in the base oil showed signs of rust within three hours.

The above tests show the remarkable rust-inhibiting and detergent-conferring properties of the additives prepared in accordance with the instant invention. Hydrocarbon oil lubricant compositions containing our new addition agents are therefore suited for use where operating conditions are extremely severe, as in diesel, tank and truck engines, and in the lubrication of steam turbines. Moreover, the addition agents of the present invention cooperate effectively with other additives. Other known addition agents which may be incorporated into lubricating compositions prepared in accordance with our invention are, for example, pour point depressants, extreme pressure agents, and the like. An oil containing a small amount of the addition agent of this invention in combination with a commercial oxidation corrosion inhibitor was tested in a Chevrolet engine. Both the piston varnish rating and the combined engine varnish and sludge rating were perfect, indicating that the detergent of the present invention does not appreciably affect the bearing corrosion value, but cooperates with the commercial corrosion inhibitor.

While we have shown in the examples the preparation of compounded lubricating oils, our invention is not limited thereto but comprises other hydrocarbon oil lubricant compositions containing our new addition agents such as greases and the like. Obviously many modifications or variations of the invention as hereinbefore set forth may be made without departing from the spirit and scope thereof and, therefore, only such limitations should be imposed as are indicated in the appended claims.

We claim:

1. A lubricant composition comprising a major amount of a hydrocarbon lubricating oil, and a minor amount, sufficient to impart rust-inhibiting properties to the composition, of a polyvalent metal salt of the condensation product of (1) an alkanethiol having 1 to 17 carbon atoms in the alkyl group and (2) a monoamide of a dicarboxylic acid wherein the two N- substituents are selected from the group consisting of hydrogen, alkyl and alkenyl radicals, at least one substituent being an organic radical of said group, and wherein the total number of carbon atoms in the N- substituents is 8 to 22, and wherein said dicarboxylic acid is selected from the group consisting of unsubstituted and alkyl-substituted 2,5-endoethylene- $\Delta^{3:4}$ -cyclohexene-1,6-dicarboxylic acids, said alkyl-substituted dicarboxylic acid having not more than four alkyl groups each having not more than 6 carbon atoms.

2. A lubricant composition comprising a major amount of a hydrocarbon lubricating oil and a minor amount, sufficient to confer detergent properties on the composition, of a polyvalent metal salt of the condensation product of (1) an alkanethiol having 1 to 17 carbon atoms in the alkyl group and (2) a monoamide of a dicarboxylic acid wherein the two N- substituents are selected from the group consisting of hydrogen, alkyl and alkenyl radicals, at least one sub-

stituent being an organic radical of said group, and wherein the total number of carbon atoms in the N- substituents is 8 to 22, and wherein said dicarboxylic acid is selected from the group consisting of unsubstituted and alkyl-substituted 2,5-endoethylene- $\Delta^{3:4}$ -cyclohexene-1,6-dicarboxylic acids, said alkyl-substituted dicarboxylic acid having not more than four alkyl groups each having not more than 6 carbon atoms.

3. A lubricant composition comprising a major amount of a hydrocarbon lubricating oil and about 0.01 to 20 per cent by weight of said oil of a polyvalent metal salt of a monoamide of a dicarboxylic acid selected from the group consisting of 2,5-endoethylene-alkyl thio-cyclohexane-1,6-dicarboxylic acids which contain not more than four alkyl groups each having not more than 6 carbon atoms, wherein the N- substituents of said monoamide are hydrogen and an alkyl radical containing 8 to 22 carbon atoms, and the alkyl thio radical contains 1 to 17 carbon atoms.

4. A lubricant composition comprising a major amount of a hydrocarbon lubricating oil, and a minor amount sufficient to impart rust-inhibiting properties to the composition, of a polyvalent metal salt of a monoamide of a 2,5-endoethylene-2-methyl-5-isopropyl-alkyl thio-cyclohexane-1,6-dicarboxylic acid wherein the N- substituents are hydrogen and an alkyl radical containing 8 to 22 carbon atoms and the alkyl thio radical contains 1 to 17 carbon atoms.

5. A lubricant composition as defined in claim 4 in which the polyvalent metal salt is a barium salt.

6. A lubricant composition as defined in claim 4 in which the polyvalent metal salt is a magnesium salt.

7. A lubricant composition comprising a major amount of a hydrocarbon lubricating oil and about 0.01 to 20 per cent by weight of said oil, of a polyvalent metal salt of a monoamide of a 2,5-endoethylene-2-methyl-5-isopropyl-alkyl thio-cyclohexane-1,6-dicarboxylic acid wherein the N- substituents are hydrogen and an alkyl radical containing 8 to 22 carbon atoms, and the alkyl thio radical contains 1 to 17 carbon atoms.

8. A lubricant composition as defined in claim 7 in which the N- substituents of the monoamide are hydrogen and a hexadecyl radical.

9. A lubricant composition as defined in claim 7 in which the N- substituents of the monoamide are hydrogen and an octadecyl radical.

10. A lubricant composition comprising a major amount of a hydrocarbon lubricating oil and about 0.01 to 20 per cent by weight of said oil, of the magnesium salt of a monoamide of 2,5-endoethylene-2-methyl-5-isopropyl-butyl thio-cyclohexane-1,6-dicarboxylic acid wherein the N- substituents are hydrogen and a hexadecyl radical.

11. A lubricant composition comprising a major amount of a hydrocarbon lubricating oil and about 0.01 to 20 per cent by weight of said oil, of the barium salt of a monoamide of 2,5-endoethylene-2-methyl-5-isopropyl-butyl thio-cyclohexane-1,6-dicarboxylic acid wherein the N- substituents are hydrogen and a hexadecyl radical.

12. A polyvalent metal salt of the condensation product of an alkanethiol containing 1 to 17 carbon atoms and a monoamide of a dicarboxylic acid selected from the group consisting of 2,5-endoethylene- $\Delta^{3:4}$ -cyclohexene-1,6-dicar-

11

boxylic acid and alkyl-substituted 2,5-endoethylene -  $\Delta^{2,4}$  - cyclohexene-1,6 - dicarboxylic acids which contain not more than four alkyl groups each having not more than 6 carbon atoms, wherein the N-substituents of said monoamide are selected from the group consisting of hydrogen and alkyl and alkenyl radicals and contain a total of 8 to 22 carbon atoms.

13. A polyvalent metal salt of a monoamide of a dicarboxylic acid selected from the group consisting of 2,5-endoethylene-alkyl thio-cyclohexane-1,6-dicarboxylic acid and alkyl-substituted 2,5-endoethylene-alkyl thio-cyclohexane-1,6-dicarboxylic acids which contain not more than four alkyl groups each having not more than 6 carbon atoms, wherein the N-substituents of said monoamide are hydrogen and an alkyl radical containing 8 to 22 carbon atoms, and the alkyl thio radical contains 1 to 17 carbon atoms.

14. A polyvalent metal salt as defined in claim 13 in which the N-substituents of said monoamide are hydrogen and a hexadecyl radical.

15. A polyvalent metal salt as defined in claim 13 in which the N-substituents of said monoamide are hydrogen and an octadecyl radical.

12

16. A polyvalent metal salt as defined in claim 13 in which the polyvalent metal is barium.

17. A polyvalent metal salt as defined in claim 13 in which the polyvalent metal is magnesium.

18. A polyvalent metal salt of a monoamide of a 2,5-endoethylene-2-methyl-5-isopropyl-alkyl thio - cyclohexane - 1,6 - dicarboxylic acid, wherein the N-substituents of said monoamide are hydrogen and an alkyl radical containing 8 to 22 carbon atoms, and said alkyl thio radical contains 1 to 17 carbon atoms.

19. A polyvalent metal salt as defined in claim 18 in which said alkyl thio radical is a butyl thio radical and said polyvalent metal is barium.

20. A polyvalent metal salt as defined in claim 18 in which said alkyl thio radical is a butyl thio radical and said polyvalent metal is magnesium.

EDWARD MITCHELL,  
WILLARD B. MORSE.

20

References Cited in the file of this patent

## UNITED STATES PATENTS

| Number    | Name     | Date           |
|-----------|----------|----------------|
| 2,408,102 | Smith    | Sept. 24, 1946 |
| 2,458,425 | Rocchini | Jan. 4, 1949   |

25